

## UNITED STATES PATENT OFFICE

2,369,656

SHALLOW HARDENING STEEL AND  
ARTICLE THEREOF

Janet Z. Briggs, New York, N. Y., assignor to  
Crucible Steel Company of America, New York,  
N. Y., a corporation of New Jersey

No Drawing. Application August 13, 1941,  
Serial No. 406,726

2 Claims. (Cl. 75—123)

This invention pertains to improvements in shallow hardening steels, and to the production and articles thereof.

The steel of the present invention is extremely shallow hardening and greatly extends the field of utility of such steels as compared to those previously known. It is particularly adapted for use in relatively thin articles requiring a glass-hard outer surface to resist wear, abrasion, penetration, etc., and a tough inner core to withstand shock, and to prevent cracking in hardening, etc., such as plow shares, small-edged cutting tools, light armor plate, etc. Heretofore, no sufficiently shallow hardening steels have been available for the production of such articles, and resort has been had to the expedients of surface hardening, viz., carburizing, nitriding, etc., or the use of composite metal for producing the same, but such expedients are both time-consuming and expensive and the results unsatisfactory. The present invention makes possible, for the first time, the production of these and like articles from shallow hardening steel with accompanying economies in time, expense and superiority of product.

Ordinary plain carbon steels are in general sufficiently shallow hardening for use in articles of relatively thick section of the order of one inch or more. For thinner sections, however, the steel either hardens throughout or the desired tough inner core is of insufficient dimension. Somewhat shallower hardening may be obtained by the additions of aluminum, or aluminum in conjunction with vanadium, whereby shallow hardening effects may be produced in sections somewhat under one inch in diameter, for example, about two-thirds inch or in rare instances, slightly less, but this has been about the lower limit heretofore obtainable.

The present invention greatly extends the previous range, and provides excellent shallow hardening in extremely thin sections of the material, of the order of about one-half to one-quarter inch or less in diameter or thickness, as well as improved effects when employed in thicker sections, as compared to existing steels.

The improvements brought about by the present invention are achieved primarily by additions of arsenic to the steel in conjunction with aluminum within specified ranges, and secondarily by restricting the upper limits of elements unavoidably present in the steel in small amounts as impurities, such as the residual metallic constituents chromium, nickel, copper, etc., the non-metallic inclusions, such as phosphorus, as well

as by restricting the upper limit of elements, such as manganese, which are added to the steel for imparting special properties thereto, such as soundness, workability, etc.

- 5 In order to secure the preferred results of the invention and to obtain the desired combination of properties in the steel, such as sufficiently shallow hardening effects, glass-like surface hardness, good core toughness, workability, etc., the 10 permissible ranges for all of the elements aforesaid are quite critical, although they may be departed from, in greater or lesser degree, particularly with increasing thickness, but at some sacrifice to the desirable characteristics.
- 15 For imparting the optimum shallow hardening properties consistent with retention of adequate workability and freedom from undue brittleness in the core, arsenic within limits of about 0.02 to 0.50% and preferably within about 0.05 to 0.30%, 20 should be employed in conjunction with a suitable deoxidizer, such as aluminum, the latter added in melting within limits of about 8 to 24 ounces per ton, and preferably within about 10 to 14 ounces per ton.
- 25 Carbon should be relatively high for imparting the desired glass-like hardness to the surface, and will ordinarily lie within the range of 0.5 to 1.5% and preferably within about 0.9 to about 1.3%.
- 30 Metallic additions, such as manganese, and residuals, such as nickel, chromium, copper, etc., are all elements which tend to impart deep hardening properties to the steel, and accordingly must be carefully restricted as to maximum content both individually and in aggregate for imparting optimum shallow hardening properties to the steel. Manganese should ordinarily be kept below about 0.5% and preferably under about 0.15% or 0.10%, although in some instances, 35 it may range as high as about 0.5 to 0.6%, depending on the thickness of section to be employed. Similarly, the residual elements, such as nickel, chromium, copper, etc., should ordinarily be held under about 0.15% and preferably under about 0.10% for the individual elements, and under about 0.45% and preferably under about 0.25% in aggregate. Such non-metallic impurities as phosphorus, etc., may be present within the usual tolerances, for example up to 0.05% of each, although it is preferred that they do not exceed about 0.03% each.
- 40 Silicon may be present within the usual tolerances of about 0.1 to 0.5% for tool steel.
- 45 A relatively broad range of analysis in accordance with the invention for imparting shallow

hardening properties particularly to thin sections of the steel, is about as follows:

|                                    |                 |
|------------------------------------|-----------------|
| Carbon—about                       | 0.5 to 1.5%     |
| Arsenic—about                      | 0.02 to 0.50%   |
| Aluminum (added in melting)—about  | 8 to 24 oz./ton |
| Manganese—about                    | 0.5% max.       |
| Silicon—about                      | 0.1 to 0.5%     |
| Nickel—about                       | 0.15% max.      |
| Chromium—about                     | 0.15% max.      |
| Copper—about                       | 0.15% max.      |
| Ni, Cr and Cu (in aggregate)—about | 0.45% max.      |
| Phosphorus                         | 0.05% max.      |
| Balance iron.                      |                 |

A preferred range for imparting somewhat shallower hardening, is the following:

|                                    |                  |
|------------------------------------|------------------|
| Carbon—about                       | 0.9 to 1.3%      |
| Arsenic—about                      | 0.05 to 0.30%    |
| Aluminum (added in melting)—about  | 10 to 14 oz./ton |
| Manganese—about                    | 0.10% max.       |
| Silicon—about                      | 0.10 to 0.25%    |
| Nickel—about                       | 0.10% max.       |
| Chromium—about                     | 0.10% max.       |
| Copper—about                       | 0.10% max.       |
| Ni, Cr and Cu (in aggregate)—about | 0.25% max.       |
| Phosphorus—about                   | 0.03% max.       |
| Sulfur—about                       | 0.03% max.       |
| Balance iron.                      |                  |

For imparting optimum shallow hardening, the following range of analysis is preferred:

|                                    |               |
|------------------------------------|---------------|
| Carbon—about                       | 1.15 to 1.25% |
| Arsenic—about                      | 0.15 to 0.25% |
| Aluminum (added in melting)—about  | 12 oz./ton    |
| Manganese—about                    | 0.05% max.    |
| Silicon—about                      | 0.1 to 0.2%   |
| Ni, Cr and Cu (in aggregate)—under | 0.25%         |
| Phosphorus—under                   | 0.03%         |
| Sulfur—under                       | 0.03%         |
| Balance iron.                      |               |

By way of illustrating the shallow hardening properties of steel in accordance with the present invention as compared to the best grades of such steels heretofore available, a round bar one-half inch in diameter and made of a steel containing about 1% carbon, about 16 ounces per ton of aluminum added in melting, manganese, residuals, phosphorus, etc., within usual tolerances, and the balance iron, was found to harden throughout on quenching from 1420° F. On the other hand, a bar of steel of similar dimensions and analysis, except for the addition of about 0.08% arsenic, was found on similar quenching to have an unhardened core of about 40% of the diameter of the bar.

The effect of the residual elements, such as chromium, nickel and copper, on the shallow hardening properties of the steel was determined by a series of tests on specimens made up in the form of slabs each  $\frac{1}{4}$  inch thick. All of these specimens were made of steels containing about 1.2% carbon, about 12 ounces per ton of aluminum added in melting, and about 0.2% arsenic, but differing, however, as regards the amounts of the residuals present. In one of the specimens, the residuals were held below the preferred limit of 0.1% for each of the elements chromium, nickel and copper, whereas in each of

the remaining specimens, this limit was exceeded for one or more of these elements. The specimen held within the above limits as to residuals was found on quenching from 1420° F. to have an unhardened core approximately one-third the thickness of the slab; whereas each of the remaining specimens hardened throughout when similarly quenched. Similar tests, however, conducted on specimens made up into thicker slabs, of the order of  $\frac{3}{4}$  inch or more, demonstrated that the effect of the residuals was relatively unimportant as regards the shallow hardening obtained. Careful regulation of the maximum residual content is therefore of controlling importance primarily in the shallow hardening of extremely thin sections of steel.

The same results were found to be true as regards variation in the manganese content. This was demonstrated by tests on a series of one-half inch round bars made of steels containing about 1.3% carbon, 0.15 to 0.25% arsenic, 12 ounces per ton of aluminum added in melting, residuals within usual tolerances, but having manganese contents of 0.33%, 0.48% and 0.71%, respectively. These analyses on quenching in circulating brine spray from 1450° F. were found to have a ratio of unhardened core to diameter of about two-thirds, one-half and zero, respectively. The tests establish, therefore, that for specimens of relatively thick dimensions, of the order of one-half inch or more, that shallow hardening is obtainable with manganese contents as high or about 0.5 to 0.6%. For thinner sections, however, the effect of manganese is more critical. This was brought out by tests on  $\frac{3}{8}$  inch slabs made of steels containing about 1.2% carbon, about 0.12% arsenic, about 12 ounces per ton of aluminum added in melting, residuals within usual tolerances, and otherwise similar analyses with the exception that one specimen contained about 0.2% manganese and the other about 0.04% manganese. The latter specimen was found on quenching from 1420° F. to have an unhardened core about one-half the thickness of the slab, whereas the specimen containing 0.2% manganese when similarly quenched, was found to harden throughout.

The effect of varying arsenic additions was demonstrated by a series of tests on one-half inch round bars made of steels of varying arsenic content but of otherwise similar analysis, viz., about 1% carbon, about 16 ounces per ton of aluminum added in melting, residuals, manganese, etc., within usual tolerances and the balance iron. These bars were found on quenching to have unhardened cores related to the arsenic content as follows:

Table I

| Arsenic addition, per cent | Ratio of unhardened core of diameter of bar |
|----------------------------|---------------------------------------------|
| About .08                  | .33                                         |
| About .20                  | .69                                         |
| About .25                  | .27                                         |

Arsenic of about 0.20%, or within the range of about 0.15 to 0.25% taking melting tolerances into consideration, is thus shown to provide optimum shallow hardening.

The effect of varying the aluminum content was demonstrated by similar tests employing one-half inch round bars each made of a steel containing

arsenic within the optimum limits of about 0.15 to 0.25%, about 1% carbon, and residuals, etc., within usual tolerances, but differing as to aluminum. These bars were found on quenching to have unhardened cores related to the aluminum addition as follows:

Table II

| Aluminum added in melting, oz./ton | Ratio of unhardened core to diameter of bar |
|------------------------------------|---------------------------------------------|
| 8                                  | 46                                          |
| 12                                 | 60                                          |
| 16                                 | 56                                          |

Thus the optimum aluminum addition is about 12 ounces per ton.

It was shown, by similar tests, that increasing additions of phosphorus noticeably impaired the shallow hardening properties of the steel, and that best results are obtained by holding these elements within the limits above stated. And the same applies as regards silicon.

The steel in accordance with the invention is preferably made from selected base material which is low in nickel, chromium, copper, phos-

phorus, and other elements, and may be produced either in the Bessemer, open hearth, the electric arc, induction or crucible furnace. The arsenic addition should be made in the furnace, and the aluminum or other deoxidizer addition in the ladle.

The steel after fabrication into articles, is preferably hardened by quenching from 1420° F., in circulating water or brine. An outstanding characteristic of the steel in this connection is that articles thereof, even in extremely thin section, may be thus shallow hardened without cracking.

I claim:

1. An alloy steel, characterized by extremely shallow hardening properties, and containing: about 0.5 to 1.5% carbon, about 0.02 to 0.5% arsenic, about 8 to 24 ounces per ton of aluminum added in melting, manganese and residual elements within commercial tolerances, and the balance substantially all iron.

2. A shallow hardened article made of an alloy steel containing: about 0.5 to 1.5% carbon, about 0.02 to about 0.5% arsenic, about 8 to 24 ounces per ton of aluminum added in melting, manganese and residual elements within commercial tolerances, and the balance substantially all iron.

JANET Z. BRIGGS.